

[54] **METHOD OF PROCESSING ANIMAL HAIR, FUR AND WOOLEN TEXTILE**[75] Inventors: **Fumio Umezawa, Tokyo; Yuji Hazaka, Fujisawa, both of Japan**[73] Assignees: **Fumikiko Umezawa; Hidefumi Umezawa, both of Tokyo, Japan**[22] Filed: **Jan. 18, 1972**[21] Appl. No.: **218,679****Related U.S. Application Data**

[63] Continuation-in-part of Ser. No. 704,520, Feb. 12, 1968, abandoned.

[52] **U.S. Cl.** ..... **8/127.51, 8/128**[51] **Int. Cl.** ..... **A61k 7/10**[58] **Field of Search** .... **8/127.51, 128, 94.14, 127.5; 252/DIG. 11, DIG. 12**[56] **References Cited****UNITED STATES PATENTS**

|           |         |                   |       |            |
|-----------|---------|-------------------|-------|------------|
| 2,382,632 | 8/1945  | Hessel et al.     | ..... | 8/128 X    |
| 2,890,926 | 6/1959  | Pardo et al.      | ..... | 8/128      |
| 3,019,171 | 1/1962  | Block et al.      | ..... | 195/68     |
| 3,059,990 | 10/1962 | Koenig et al.     | ..... | 8/128      |
| 3,079,213 | 2/1963  | Mendelsohn et al. | ..... | 8/128 X    |
| 3,193,463 | 7/1965  | Schweizer         | ..... | 8/127.51 X |
| 3,266,994 | 8/1966  | Reiss et al.      | ..... | 8/127.51   |
| 3,472,783 | 10/1968 | Smillie et al.    | ..... | 252/89     |

**FOREIGN PATENTS OR APPLICATIONS**

282,588 5/1927 Great Britain ..... 252/DIG. 12

1,033,229 6/1966 Great Britain ..... 252/DIG.12

**OTHER PUBLICATIONS**

Cadwell et al., "The Mechanism of Setting of Wool in Alkaline Solutions," Textile Research Journal, Nov. 1964, pp. 933-939.

Roberts et al., "Basic Principles of Organic Chemistry," 1965, pp. 725-726.

Schwartz et al., "Surface Active Agents and Detergents," Vol. II, 1958, pp. 381-382.

Martell et al., Chemistry of the Metal Chelate Compounds, 1952, pp. 401-405 and 510-511.

Sotiriou-Provata et al., "The Setting Characteristics of Metal-Containing Wool Fibers," Textile Research Journal, June 1965, pp. 578-579.

Whewell et al., "The Action of Copper Amines on Wool," The Textile Research Journal, May 1959, pp. 386-393.

**Primary Examiner**—Thomas J. Herbert, Jr.**Attorney, Agent, or Firm**—William J. Daniel[57] **ABSTRACT**

A process for setting animal hair material by first treating the material with an alkaline solution and then with an aqueous solution of a water-soluble compound of a metal forming a colorless complex with the animal hair, such as calcium, aluminum, lanthanum and zirconium.

**5 Claims, 1 Drawing Figure**

PATENTED OCT 8 1974

3,840,401



## METHOD OF PROCESSING ANIMAL HAIR, FUR AND WOOLEN TEXTILE

This application is a continuation-in-part of application Ser. No. 704,520 filed February 12, 1968, now abandoned.

This invention relates to a process for setting of animal hair goods, more specifically, to a process for setting of animal hair goods by treating the animal hair in two stages treatment under a mild treating condition to provide the setting of the animal hair goods without injuring the inherent desirable properties of the animal hair.

Heretofore, as to the process for setting of animal hair goods such as woolen textile, such process as heat setting process using steam or hot water, or chemical setting process using thioglycolate and bromide in combination, or persulfate, has been already known. These known processes are conducted for the purpose of preventing crimp of animal hair which is inherent to the animal hair, or which would be given during the any given stages of processing of the hair for the final product from raw material. Said known processes are also conducted for the purpose of setting pleats on the woolen textile.

As far as the fur is concerned, said known setting processes using steam, hot water, thioglycolate and bromide, etc., are not able to employed, for those processes might cause undesirable results of changing texture of fur, removing hair from fur, and degrading skin of fur. Accordingly, for setting fur, it is employed such process as coating the fur with protective material such as glycerin, arranging the lie of hair and then pressing the fur.

The hair of fur, especially coarse hair has a tendency of easy to crimp in natural condition, and it is apt to crimp especially in a course of dyeing. As the results of said tendency, quality of the fur may be remarkably degraded due to angle like shape crimp formed at the tip of hair, or irregular wave like pattern formed on the whole surface of the fur. Said tendency of the fur is especially noticeable in the case of fur of fox.

As said above, the known setting process is able to carried relatively easy, but is accompanied by undesirable effect of degrading the animal hair goods.

Another process also has been known for shrink-proofing and feltpoofing of sheep wool. The said process comprises treating the sheep wool with alkaline solution and then treating it with chromium complex salt of carboxylic acid. However, the process provides the intended effect but the process is not satisfactorily employed as the commercial process, for it causes coloring of the treated sheep wool due to the color of chromium ion.

Accordingly, an object of this invention is to provide an effective setting process of animal hair goods including animal hair, fur and woolen textile, without injuring inherent properties of animal hair such as feeling, texture, color etc.

The other object of this invention is to provide a process for forming a stable chelate compound of keratin protein of animal hair and heavy metal, by arranging the configuration of the keratin protein molecule so as to make the keratin easy to form the chelate compound with the heavy metal, and then reacting so arranged keratin protein with an aqueous solution of the water soluble heavy metal salt.

Another object of this invention is to provide a composition utilized for rearranging the configuration of keratin protein and forming the chelate compound of the keratin and heavy metal at the same time.

5 Further object of this invention will be obvious from the description hereinafter.

It has been found that the animal hair goods may be set without injuring the inherent properties of the animal hair, by treating the animal hair goods with an aqueous solution containing at least one of alkaline substance selected from the group consisting of hydroxide, carbonate and bicarbonate of sodium, potassium and ammonium and lower alkanol amine, and then treating further with an aqueous solution of water soluble metal compound of a metal selected from the group consisting of calcium, tin, aluminum, lanthanum, and zirconium.

Further it has been found that the animal hair goods may easily be set up in the single step treatment using an aqueous solution containing the first constituent selected from the group consisting of hydroxide, carbonate and bicarbonate of sodium, potassium and ammonium, and lower alkanol amine, and the second constituent selected from the group consisting of water soluble compounds of calcium, tin, aluminum, lanthanum and zirconium, in the presence of a complex compound forming substance having less complex-forming capability than the keratin protein molecule, such as amino acid, peptide and enzyme.

Still further, it has been found that said setting of the animal hair goods may be conducted more effectively by incorporating into said treating solution nonionic or anionic surface active agent.

35 The process of this invention comprises: treating animal hair goods with an aqueous solution containing at least one of compound selected from the group consisting of hydroxide, carbonate and bicarbonate of sodium, potassium and ammonium, or at least one of lower alkanol amine, to rearrange the configuration of the keratin protein of animal hair and to make easy the formation of chelate compound with the metal compound used, in the first stage of the process; and further treating with an aqueous solution of water soluble compound of a metal selected from the group consisting of calcium, tin, aluminum, lanthanum and zirconium, so as to form chelate compound with the keratin having rearranged configuration and the metal, in the second stage of the process.

50 The treating solution used in the first stage of this process is the aqueous solution containing at least one of the alkaline substances selected from the group consisting of hydroxide, carbonate, and bicarbonate of sodium, potassium and ammonium, or at least one of lower alkanol amine such as monoethanol amine, diethanol amine, and triethanol amine, in a concentration of the range from 0.1 to 5% by weight. When the concentration of the alkaline substance in above solution is less than 0.1% by weight, insufficient rearrangement

55 of the configuration of keratin molecule is obtained, while said concentration is more than 5% by weight, the desirable properties of resulting animal hair goods are injured. Therefore, the concentration of the alkaline substance used should be in above range. Further, in order to conduct the first stage treatment effectively, it is necessary to adjust the pH of the solution in the range from 9.0 to 10.5.

The treatment of the animal hair goods in the first stage is conducted by contacting the animal hair goods with the treating solution at a temperature of 30°-60°C for a period of 3 - 10 minutes. When the treatment is conducted at a temperature below 30°C or for a period of less than 3 minutes, excellent set is not achieved due to the insufficient rearrangement of configuration of the keratin protein molecule. While, where said the first stage treatment is carried at a temperature above 60°C or for a period of more than 10 minutes, the animal hair is injured and degraded.

Into said first stage treating solution, it is preferred to add nonionic or anionic surface active agent in an amount of the range from 0.5 to 3% by weight, for said surface active agent added accelerates the rearrangement of the configuration of the keratin molecule. As said nonionic or anionic surface active agent, sulfuric acid ester of higher alcohol, polyoxy alkylene ether, polyoxy alkylene ester and the like are preferred. The cationic surface active agent can not be used in this process as it forms precipitation together with metal ion used in the next stage of the treatment. Into the treating solution, a buffer agent such as sodium phosphate, may further be added.

By the first stage treatment of the animal hair goods, it is estimated that the keratin protein of the animal hair would take sodium, potassium or substituted or unsubstituted ammonium ion into its molecule, and form transient bond between the protein and the ion in such a manner as the configuration of the molecule be rearranged to make easy the formation of chelate compound.

The treating solution used in the second stage of this process to form chelate compound, is an aqueous solution containing water soluble compound of calcium, tin, aluminum, lanthanum or zirconium. Illustrative water soluble compounds of said metals include: chloride, sulfate, hydroxide and organic acid salt of said metals, such as calcium chloride, tin chloride, aluminum chloride, calcium oxide, calcium hydroxide, lanthanum chloride, and zirconium acetate. The concentration of the said compound in the aqueous solution is not critical, but generally is selected from the range of 0.1 to 5% by weight.

The animal hair goods treating temperature in the second stage of this process is in the range of from 30° to 50°C, and from 3 to 10 minutes treatment is sufficient as the treating period. The bath ratio, i.e., the ratio of the weight of the treating solution to the weight of the animal hair goods is in the range of about 1 : 30 - 50. Into the treating solution used in the second stage of this process, nonionic or anionic surface active agent may further be added so as to accelerate the setting of the animal hair goods. Said surface active agent may be added in an amount of the range from 0.5 to 3% by weight.

By the said treatment of the second stage of the process, it is estimated that the chelate structures are formed through the bondage of the metal ions used and lone pair electron having atoms such as sulfur, nitrogen and oxygen in the keratin protein of the animal hair. When the said chelate structure is related with nitrogen atoms and the metal, the following structural formula is estimated:



wherein

R, R' and R'' stand for amino acid residues. As said above, in the process of this invention, it is necessary to use two of treating solution in principle, one of which is the solution containing alkaline substance for the purpose of rearranging the configuration of the keratin molecule, and the other is the solution containing metal ion for the formation of chelate compound. If the animal hair goods is treated using a single solution containing both said alkaline substance and metal ion, one can not obtain the desired setting effect. However, if a single complex solution containing said alkaline, metal ion, and further a complex compound forming substance which has less chelate-forming capability than keratin, such as amino acid, peptide and enzyme, is used as the treating solution, one can conduct both the rearrangement of the configuration of the keratin molecule and the formation of the chelate compound in a single step of the treatment. As the treating solution for this single step treatment, such an aqueous solution containing at least one of alkaline substance selected from the group consisting of hydroxide, carbonate and bicarbonate of sodium, potassium and ammonium, or at least one of lower alkanol amine, in an amount of 0.1 - 5% by weight, a compound selected from the group consisting of water soluble compound of calcium, tin, aluminum, lanthanum and zirconium, in an amount of 0.1 - 5% by weight, and a stabilizer selected from the group consisting of amino acid, peptide and enzyme, in an amount of 0.1 - 1% by weight, is preferred. Further into the solution, above-stated nonionic or anionic surface active agent, and above-stated buffer agent may also be incorporated. The animal hair goods treating condition using the single treating solution, is almost identical with the said two treating solution process, except a somewhat longer treating time is used.

The animal hair goods so treated in accordance with the process of this invention, are then washed in several times by warm water of 30°- 50°C or more, soaped by using a nonionic or anionic surface active agent solution of 0.1 - 0.5% concentration, rinsed again by water completely, and then dried at a mild temperature of less than 100°C. In this manner, the animal hair goods having substantially the same color, luster, and feeling as the untreated animal hair goods, but having an excellent setting effect, are obtained.

It is observed that many of animal hair goods once set by the conventional process, are easily deformed when they are immersed in a hot water of 50°C for a few minutes, while the animal hair goods being set in accordance with this process, are not deformed but kept their set form even after immersing them into a hot water of 95 - 100°C for more than 10 minutes.

Where it is desired for some reasons or other, to release the set form of the set-treated animal hair goods obtained by this process into the original form of them, one can treat them with a solution containing 0.1 - 2% of chelating agent such as sodium ethylene diamine tetraacetate, 8-oxyquinoline, nitrilo triacetic acid and the like, to decompose the chelate structure of keratin

molecule, and the set form is easily converted into the original form of the hair. In the above case, the animal hair goods are treated at a temperature higher than the setting temperature for a period of time from 2 to 20 minutes.

In accordance with the process of this invention, as the setting of the animal hair goods is conducted in a mild condition with effective setting result, that the treatment does not injure the animal hair goods themselves and also inherent properties of them.

The invention is further demonstrated by the following examples, which are given merely by the way of illustration and not limitation. In the following example, all parts or percentage are given by weight. In the following example, set efficiency is determined in the manner detailed below;

Sample yarn of  $L$  mm length is wound on a glass rod of 3.5 mm in diameter, and the so wound yarn is set-finished. Then the length of so set-finished yarn is measured. When found length is  $L'$  mm, the apparent set efficiency  $E$  is obtained by the following formula:

$$E = L - L'/L \times 100$$

So set-treated yarn is then heat-treated in hot water of 70°C for 10 minutes. After that length of yarn so treated is measured. When found length of yarn is  $L''$ , the true set efficiency  $E'$  is obtained by the following formula:

$$E' = L - L''/L \times 100$$

#### Example 1.

Two of the treating solutions having the following composition were prepared:

##### The first treating solution:

Triethanol amine 0.5 parts  
Sodium lauryl sulfate 0.3 parts  
Water balance(to give 100 parts of solution)

##### The second treating solution:

Calcium oxide 1 part  
Polyoxyethylene laurate 0.5 parts  
Disodium hydrogen phosphate 0.3 parts  
Water balance(to give 100 parts of solution)

Wool yarn was wound around a glass rod, and was immersed in the first treating solution heated at about 40°C for 3 minutes. Then so treated wool yarn was immersed in the second treating solution heated at about 40°C for 5 minutes, washed with water, soaping-treated in the known manner and then dried. In this manner the wool yarn being set-finished in spiral form was obtained. The yarn so obtained had the same color, texture and feeling as the untreated yarn.

Then the apparent and true set efficiency of so set-finished wool yarn, and of wool yarn being set-finished in conventional manner of heating the yarn at 120°C for 5 minutes in air, were determined and compared. The results obtained are shown in the following table:

| No. | Sample                                    | Apparent set efficiency | True set efficiency |
|-----|-------------------------------------------|-------------------------|---------------------|
| 1   | Wool yarn treated by this process         | 70%                     | 65%                 |
| 2   | Wool yarn treated by conventional process | 75%                     | 37%                 |

Then the elongation-load curve of said samples were determined. The results are shown in FIG. 1.

As apparent from said results, the wool yarn being treated in accordance with this process has bigger strength and elongation than the wool yarn being treated by the conventional process.

#### Example 2.

In this example, two of the treating solutions having the following composition, were prepared:

##### The first treating solution:

Disodium hydrogen phosphate 1.0 part  
Sodium hydroxide 0.1 part  
Diethanol amine salt 0.3 parts  
of lauryl sulfate  
Water

balance(to give 100 parts of solution)

##### The second treating solution:

Stannic chloride 0.3 parts  
Polyethylene alkyl ether 0.2 parts  
Water

balance(to give 100 parts of solution)

Wool cloth was immersed in the first treating solution heated at about 40°C for 3 minutes, squeezing off the solution from the cloth, and then the cloth was folded and pleated. So pleated cloth was then immersed in the second treating solution heated at about 40°C for 1 minute, washed with water, and soaping treated. After drying, the set cloth having pleats was obtained. There was no change in color of the so obtained cloth compared with the untreated cloth.

The set efficiency of so treated cloth, together with of the cloth being set only by using the second treating solution, for the comparison, were determined. The results obtained are shown in the following table:

| No. | Sample                                           | Apparent set efficiency | True set efficiency |
|-----|--------------------------------------------------|-------------------------|---------------------|
| 1   | Wool cloth treated by this process               | 63%                     | 55%                 |
| 2   | Wool cloth treated by only 2nd treating solution | 25%                     | 0%                  |

#### Example 3.

Fur of mutton was treated with 3% aqueous solution of monoethanol amine at 40°C for 3 minutes in the first place. Then the fur was brushed to stretch out the crimples of the hair and to arrange the lie of the hair of the fur. Onto so treated fur, a paste consisting of 0.5 parts of aluminum potassium sulfate, 0.2 parts of alkylol amide, 6 parts of carboxymethyl cellulose and 93.3 parts of water, was coated. The paste coated fur was steam-treated for 2 minutes. Then the fur was soaping-treated, washed to remove the paste and dried. In this manner, crimped hair of the fur was able to stretch out without spoiling and injuring the fur.

#### Example 4.

In this example, two of the following treating solutions having the following composition, were prepared:

##### The first treating solution:

Monooethanol amine 0.5 parts  
Alkylol amide 0.5 parts  
Water

balance(to give 100 parts of solution)

## -Continued

## The second treating solution:

|                             |                                        |
|-----------------------------|----------------------------------------|
| Zirconium acetate           | 0.1 part                               |
| Diethanol amine             | 0.3 parts                              |
| Polyoxyethylene alkyl ether | 0.3 parts                              |
| Water                       | balance(to give 100 parts of solution) |

Wool yarn was set as the same manner described in the Example 1, by treating it with the first treating solution heated at about 35°C for 5 minutes, and then treating it with the second treating solution heated at about 55°C for 5 minutes. Then the yarn was washed and dried as the same manner as the Example 1. So obtained wool yarn had the true set efficiency of 55%.

## Example 5.

Wool cloth was treated as the same manner described in the Example 2, but treating it with the first treating solution heated at 40°C for 5 minutes, and the second treating solution heated at 40°C for 7 minutes, and set cloth having the true set efficiency of 60% was obtained. The first and second treating solution here used having the following composition:

## The first treating solution:

|                                        |                                        |
|----------------------------------------|----------------------------------------|
| Monoethanol amine                      | 0.3 parts                              |
| Ammonium carbonate                     | 0.5 parts                              |
| Diethanol amine salt of lauryl sulfate | 0.3 parts                              |
| Water                                  | balance(to give 100 parts of solution) |

## The second treating solution:

|                             |                                        |
|-----------------------------|----------------------------------------|
| Lanthanum chloride          | 0.5 parts                              |
| Polyoxyethylene alkyl ether | 0.2 parts                              |
| Water                       | balance(to give 100 parts of solution) |

## Example 6.

Into an aqueous solution containing 1.5% glycine and 0.5% zirconium acetate, sodium carbonate was added to adjust the pH of the solution to 10. Into the solution, wool cloth previously finely pleated was immersed at 45°C for 10 minutes. So treated cloth was washed with hot water, soaping-treated and dried to give finely pleated cloth. The cloth had the true set efficiency at 71%.

## Example 7.

Into an aqueous solution containing 2% amylase, and 0.5% aluminum potassium sulfate, monoethanol amine was added to adjust the pH of the solution to 8. Into the solution, hair of yak, being coiled on glass rod, was immersed while maintaining the solution at 40°C. After 5 minutes, the hair was taken out from the solution, washed with hot water, soaping-treated, and then dried. In this manner the hair of yak was set in spiral form without injuring the hair which is known very fragile to alkali.

We claim:

1. A process for setting textile material formed of animal hair which comprises: arranging said textile material in a predetermined configuration and while maintaining said configuration, first treating the animal hair goods with an aqueous solution consisting essentially of at least one of alkaline substances selected from the group consisting of hydroxide, carbonate and bicarbonate of sodium, potassium and ammonium, and lower alkanol amines in a concentration of the range from 0.1 to 5% by weight, said solution being adjusted to a pH of the range from 9.0 to 10.5, in the first stage treatment; and then treating the thus treated animal hair goods with an aqueous solution consisting essentially of

10 a water soluble salt with an organic or carboxylic acid of a heavy metal selected from the group consisting of calcium, aluminum, tin, lanthanum and zirconium forming a colorless complex with said animal hair.

2. A process for setting textile material formed of ani-

20 mal hair which comprises: arranging said textile material in a predetermined configuration and while maintaining said configuration, treating the animal hair goods with an aqueous solution consisting essentially of at least one of alkaline substances selected from the group consisting of hydroxide, carbonate and bicarbonate and sodium, potassium and ammonium, and lower alkanol amines in a concentration of the range from 0.1 to 5% by weight; a water soluble salt with an inorganic or carboxylic acid of a heavy metal forming a colorless

25 complex with said animal hair, in a concentration of the range from 0.1 to 5% by weight; and at least one of stabilizer compounds selected from the group consisting of amino acid, peptide and enzyme in a concentration of the range from 0.1 to 1% by weight.

3. The process of claim 2 wherein said heavy metal is selected from the group consisting of calcium, aluminum, tin, lanthanum and zirconium.

4. A composition for setting textile material formed of animal hair consisting essentially of (1) at least one alkaline substance selected from the group consisting of hydroxide, carbonate and bicarbonate of sodium, potassium and ammonium, and lower alkanol amines, (2) a water soluble salt with an inorganic or carboxylic acid of a heavy metal forming a colorless complex with said animal hair, and (3) at least one stabilizer compound selected from the group consisting of amino acid, peptide and enzyme.

5. The composition of claim 4 wherein said heavy metal is selected from the group consisting of calcium, aluminum, tin, lanthanum and zirconium.

\* \* \* \* \*

UNITED STATES PATENT OFFICE  
CERTIFICATE OF CORRECTION

Patent No. 3,840,401 Dated October 8, 1974

Inventor(s) Fumio UMEZAWA et al

It is certified that error appears in the above-identified patent and that said Letters Patent are hereby corrected as shown below:

In the Heading of the Patent, insert

-- [30] Foreign Application Priority Data

February 18, 1967...Japan...10320/1967

Signed and sealed this 4th day of March 1975.

(SEAL)

Attest:

RUTH C. MASON  
Attesting Officer

C. MARSHALL DANN  
Commissioner of Patents  
and Trademarks